

1

2,827,433

## EXTREME PRESSURE LUBRICANT COMPOSITION

Fred B. Fischl, Springfield, and Walter E. Waddey and Fred J. Beyerstedt, Westfield, N. J., assignors to Esso Research and Engineering Company, a corporation of Delaware

No Drawing. Application March 11, 1954  
Serial No. 415,692

1 Claim. (Cl. 252—46.7)

The present invention relates to improved extreme pressure lubricant compositions and the like. It particularly relates to oils, greases and other compositions used in heavy duty lubricant service, which contain an improved combination of additive materials.

Briefly, the present invention contemplates a lubricant composition comprising a minor portion of a combination additive including a phosphorus and sulfur-containing hydrocarbon and a sulfur and halogen-containing organic compound.

It is known to compound lubricants with phosphosulfurized hydrocarbons, such as  $P_2S_5$ -treated mineral lubricating oils to form compositions useful in heavy duty service, particularly where unit loads are exceptionally high, as for example in automotive differential units and hypoid gearing. These compositions are particularly effective in high torque-low speed gear operation, but their performance is from borderline to unsatisfactory in low torque-high speed gear operation. Because this deficiency has been recognized, various procedures have been employed for improving these compositions in this respect. These procedures include treatment of the additive with various substances, blending other types of agents in the composition, and the like. None of the solutions attempted heretofore have provided a complete answer to the problem. However, in view of the availability and low cost of the phosphosulfurized materials, and their excellence in other respects for this type of service, a satisfactory means for overcoming this deficiency has been needed.

In accordance with this invention, it has been found that the extreme pressure characteristics of lubricants containing phosphosulfurized hydrocarbons is significantly improved, particularly with respect to low torque-high speed operation by the addition thereto of a relatively small amount of a halogen and sulfur-bearing organic compound, such as a halohydrocarbon sulfide. Preferably, in accordance with this invention, the concentration of the phosphosulfurized hydrocarbon is substantially in excess of that of the halogen and sulfur-containing compound in order to also insure satisfactory high torque-low speed performance.

It has been found that lubricants compounded with these two types of additives demonstrate unexpectedly superior extreme pressure performance in contrast to the predicted performance based on the effect exerted by each of the additives when used alone in the same lubricant base stock. Furthermore, the finished compositions compounded in accordance with this invention are superior in high speed-low torque extreme pressure service, and pass the rigid requirements imposed by U. S. Government specifications in this test.

The results obtained in the practice of this invention are unexpected from several standpoints. While it is well-known in the art to employ various halogenated organic compounds as additives in extreme pressure service, it was found that typical members of this class do not improve sufficiently to meet the high speed-low torque

2

test, either when the halogenated materials were used alone or in combination with phosphosulfurized hydrocarbons. It is indeed surprising to find that halogenated compounds containing sulfur contributed a synergistic extreme pressure improvement to the phosphosulfurized hydrocarbon,

particularly when the former material is used in concentrations at which it normally imparts very little or no extreme pressure properties in ordinary lubricant base stocks. The reasons for these unexpected results cannot

be explained at this time.

In the first step of the preparation of the phosphosulfurized additives employed in accordance with the present invention, a sulfide of phosphorus is reacted with a hydrocarbon material. The sulfide of phosphorus which can

be employed includes  $P_2S_3$ ,  $P_2S_5$ ,  $P_4S_3$ ,  $P_4S_7$  or other phosphorus sulfide, and is preferably phosphorus pentasulfide ( $P_2S_5$ ). Mixtures of two or more phosphorus sulfides may also be employed as well as mixtures of elemental phosphorus and sulfur.

The hydrocarbon materials which may be reacted with a phosphorus sulfide may be paraffins, olefins, or olefin polymers, diolefins, acetylenes, aromatics or alkyl aromatics, cyclic aliphatics, petroleum fractions, such as lubricating oil fractions, petrolatums, waxes, cracked cycle stocks, or condensation products of petroleum fractions, solvent extracts of petroleum fractions, etc.

As examples of monoolefins may be mentioned isobutylene, decene, dodecene, cetene ( $C_{16}$ ), octadecene ( $C_{18}$ ), cerotene ( $C_{20}$ ), melene ( $C_{30}$ ), olefinic extracts from gasoline

line or gasoline itself, cracked cycle stocks and polymers thereof, resin oils from crude oil, hydrocarbon coil resins, cracked waxes, dehydrohalogenated chlorinated waxes, and any mixed high molecular weight alkenes obtained by cracking petroleum oils.

Another class of suitable olefinic materials are the monoolefin polymers, in which the molecular weight ranges from 100 to 50,000, preferably from about 250 to about 10,000. These polymers may be obtained by the polymerization of low molecular weight monoolefinic hydrocarbons, such as ethylene, propylene, butylene, isobutylene, normal and isomethylenes, or hexenes, or by the copolymerization of any combination of the above monoolefinic materials.

Another class of hydrocarbons which may be employed in a similar manner are aromatic hydrocarbons, such as benzene, naphthalene, anthracene, toluene, xylene, diphenyl, and the like, as well as aromatic hydrocarbons having alkyl substituents and aliphatic hydrocarbons having aryl substituents.

Another type of hydrocarbon material which may be similarly employed is a resin-like oil which has a molecular weight of from about 1,000 to 2,000 or higher, obtained preferably from a paraffinic oil which has been dewaxed and which is then treated with a liquified normally gaseous hydrocarbon, e. g. propane, to precipitate a heavy propane-insoluble fraction. The latter is a substantially wax-free and asphalt-free product having a Saybolt viscosity at 210° F. of about 1,000 to about 4,000 seconds or more.

The phosphorus sulfide-hydrocarbon reaction product may be readily obtained by reacting the phosphorus sulfide with the hydrocarbon at a temperature of about 200° F. to about 600° F., and preferably from about 300° F. to about 550° F., using from about 5% to about 25%, preferably about 10% to about 20% by weight of phosphorus sulfide based on hydrocarbon. It is advantageous to maintain a non-oxidizing atmosphere, such as an atmosphere of nitrogen, above the reaction mixture. Usually it is desirable to use an amount of the phosphorus sulfide

that will completely react with the hydrocarbon so that no further purification becomes necessary. In the case of monoolefin polymers the preferred ratio is one molecular

proportion of the sulfide of phosphorus to two to five molecular proportions of polymer. In such case the reaction is continued until all or substantially all of the phosphorus sulfide has reacted. The reaction time is not critical, and the time required to cause the maximum amount of phosphorus sulfide to react will vary with the temperature. A reaction time of two to ten hours is frequently necessary.

Although the resulting acidic phosphosulfurized product may be used as such, it is preferred to refine it further in order to improve odor, anti-corrosive, extreme pressure, detergency, stability and other properties. Such refining procedures are well known to the art, and include blowing with steam, alcohols, phenols, and the like at elevated temperature of about 200° to 600° F., reacting with various metal and ashless basic reacting agents, treating with olefinic hydrocarbons, etc.

Thus, metallic treating agents include the alkali metal and alkaline earth metal oxides, hydroxides, hydrides and the like, specifically such compounds of potassium, sodium, barium, and calcium.

Suitable ashless treating agents include nitrogen bases such as ammonia, and organic nitrogen bases such as amines and amine derivatives, guanidines and their derivatives, morpholine, pyridine, quinoline and like substances. Guanidine and its derivatives are particularly useful, the symmetrical tri-substituted compounds, such as trialkyl and triphenyl guanidines and the like being useful. Other useful compounds include the biguanides, dicyandiamides, dicyandiamides, hydrazines, ureas, thioureas, semicarbazides, thiosemicarbazides, maleate and fumarate esters, aminoalcohols, acrylonitrile, alcohols, vinyl esters, phenols, olefins such as diisobutylene, dipentene, and the like. Such treating agents are disclosed in the art such as U. S. Patents 2,613,205; 2,640,030; and 2,640,053.

Treatment of the product with these and other agents may be carried out at any suitable temperature, such as from about room temperature up to 400° F. or so using sufficient treating agent at least to partially neutralize, esterify or combine with the titratable acidity of the phosphosulfurized material. Completely neutralized materials are usually preferred.

A particularly desirable method for reducing H<sub>2</sub>S evolution and improving odor is that of following the teachings of U. S. Patent 2,640,053 in which the phosphosulfurized hydrocarbon is treated with about 0.1 to 50% of its weight of an olefinic hydrocarbon.

The preferred olefinic hydrocarbon materials to be reacted with the phosphosulfurized material includes the terpenes, such as turpentine, dipentene, alpha-pinene, terpinene, terpineol, and the like and such olefinic hydrocarbons as isobutylene, diisobutylene, and the more reactive of the analogous aliphatic and cycloaliphatic materials.

In particular, a product sold commercially as "Dipentene" consisting primarily of a mixture of true dipentene with its isomers and minor proportions of related products, is used in proportions of about 2 to 30% by weight based on the material to be treated, the ingredients being mixed together and heated at a suitable temperature until the product is stabilized. Preferred proportions are 5 to 15% by weight. Stability is indicated by reduced evolution of H<sub>2</sub>S gas at ordinary temperatures and at moderately elevated temperatures such as 150° or even up to 400° F. The soaking temperature and the soaking time will vary depending upon the particular ingredients and upon the degree of stability required. In general the invention contemplates a range of soaking temperatures from as low as 60° to as high as about 400° F. The soaking time may be from 1 to 10 hours, depending upon the tendency to evolve H<sub>2</sub>S gas and upon the degree of stability desired.

It may also be desired to improve the stability of the phosphosulfurized product and to reduce its sludge-forming characteristics by inhibiting it with a small amount

of a soluble metal petroleum sulfonate and a metal alkyl phenol sulfide. The sulfonates may be an alkali or alkaline earth salt, including the lithium, sodium, potassium, calcium, strontium, and barium salts of the hydrocarbon sulfonates prepared by the treatment of petroleum oils with strong sulfuric acid followed, for example, by treatment with a base of the metal. The alkali or alkaline earth metal sulfonates are most commonly used, but petroleum sulfonates of other metals may be used if they are soluble in the lubricant in the small concentrations required in the practice of the present invention. Mixtures of the various sulfonates may be employed if desired. Preferably the sodium and calcium sulfonates are used. The most effective sulfonates are those having relatively high molecular weights such as from about 400 for monovalent to about 1100 for divalent salts. The sulfonates are generally added to the phosphosulfurized additive in concentrations ranging from 0.02 to 1.0 weight percent with preferred concentrations ranging from 0.05 to 0.3 weight percent.

The alkaline earth metal salts of alkyl phenol sulfides include those in which the alkaline earth metals are calcium, barium, strontium, and magnesium. The presence of at least one alkyl group in the benzene nucleus is usually desirable to impart oil solubility to the compound. The alkyl group may contain from 4 to 12 or more carbon atoms and may be straight chain or branched. From one to four sulfur atoms may interconnect benzene nuclei. The sulfide may contain only one alkaline earth metal or may have a mixture of at least two alkaline earth metals in the same molecule. Barium is generally the preferred metal, calcium being second choice, as a rule. The concentration of the alkyl phenol sulfide salt is usually in the range of 0.05 to 2.0%, preferably in the range of about 0.1 to 1.0% by weight based on the treated phosphosulfurized oil. The weight ratio of petroleum sulfonate to alkyl phenol sulfide salt is preferably in the range of 1:1 to 1:3.

The phosphosulfurized additive may be used in various proportions in lubricants depending upon the specific application. In the lubrication of automotive hypoid gears, a concentration of about 3 to 20 weight percent, preferably 5 to 15% and especially 8 to 12%, based on the total lubricant is used to impart substantial high torque extreme pressure properties to the lubricant.

The sulfur- and halogen-containing organic compound used in combination with the phosphosulfurized hydrocarbon is preferably a halo-hydrocarbon sulfide, such as a mono-, or di-, or poly sulfide. Since the aromatic derivatives, such as for example, the chlorinated and brominated alkaryl sulfides, are generally more stable and therefore less corrosive than the sulfohalogenated aliphatic compounds the former are especially preferred. However, for some uses, sulfochlorinated hydrocarbons such as those formed by treating olefins, paraffins, naphthenes and the like, with sulfur halides may be used. Thus, the reaction product of sulfur chloride and paraffin wax, or mixtures of wax and kerosene may be employed.

Other useful materials may be prepared by treating chlorinated hydrocarbons, such as chlorinated kerosenes, gas oils, mineral lubricating oil distillates, waxes, etc., with an inorganic polysulfide such as a sodium polysulfide whereby a portion of the chlorine is replaced with sulfur to form chlorohydrocarbon sulfides. Aromatic hydrocarbons, such as alkyl aromatics, may be prepared by prior art processes in which halogen is first introduced into the benzene ring, and then into the alkyl groups. Two of the resulting molecules may then be joined by replacing the alkyl halogen atoms with one or more sulfur atoms by treatment with an alkali metal sulfide to form the haloalkyl sulfide.

In another procedure, a mixture of benzyl chlorides and chlorobenzyl chlorides, for example, may be reacted with a metal sulfide to form useful mixed compounds.

Such processes are well known to the art, and need not be discussed in detail herein.

Specific useful halohydrocarbon sulfides include chloroparaffin wax polysulfide, dibromodiphenyl disulfide, dichlorodibenzylsulfide, chlorodimethylbenzyl disulfide, and the like. The halogen-containing dibenzyl disulfides, such as chlorodibenzyl disulfide, are especially preferred.

The amount of the chlorine and sulfur-containing compound used in conjunction with the primary additive may vary widely. Generally, it is used in amounts ranging from about 0.1 to 10% by weight based on the total oil, preferably about 0.3 to 5%, and especially 0.5 to 2.0% at concentrations less than the concentration of phosphosulfurized hydrocarbon used. Thus, weight ratios of phosphosulfurized hydrocarbon to the halogen- and sulfur-containing hydrocarbon in the range of 2:1 to 30:1, especially 5:1 to 20:1, are useful.

The additives of the present invention may be employed not only in ordinary oil-base lubricants, but especially find application in "heavy duty" types of lubricants that have been compounded with detergent additives such as metal soaps and the like, dyes, pour depressors, antioxidants, viscosity index improvers, thickeners, corrosion inhibitors, etc. Suitable base stocks include animal, vegetable and mineral and synthetic oils. Preferably, they are mineral oils that have been refined by usual procedures, including acid and/or alkali treatment, solvent extraction, etc., although other oleaginous base stocks may be used.

For example, synthetic oils, including polymerized olefins, cracking coil tar fractions, animal, vegetable or fish oils or their hydrogenated products, etc., may be used alone or in admixture with mineral oils. Synthetic oils of the ester, polyester, polyether and related types may be used. These include di-2-ethyl-hexyl sebacate, dibasic acid esters, polyalkylene oxides, etc. Especially suitable, however, are the high viscosity mineral oils having utility in extreme pressure service such as those having SSU viscosities at 210° F. of 50 to 150 or higher, and soap thickened greases prepared from mineral oils and the like.

Various modes of practicing this invention are specifically illustrated in the following examples:

## EXAMPLES

### I. Description of additives

*Additive A.*—A deasphalted, dewaxed, acid- and clay-treated Panhandle mineral oil bright stock having an S. U. S. viscosity of 170 at 210° F. was treated in a nitrogen atmosphere with about 17% by weight, based on the oil, of  $P_2S_5$  for about 10 hours at a temperature of about 425° F. The product was filtered, and was then treated with 9.5 weight percent of commercial dipentene and 1.0 weight percent of a stabilizer at a temperature of about 380° F. with stirring for one hour.

The commercial dipentene employed contained about 31% dipentene, 39% terpinolene, 6% alpha-pinene, 10% para-cymene, 7% alpha terpeneol, 5% 2,4(8)-p-methadiene, and 2% residue.

The stabilizer employed was a blend containing about 33 weight percent of sodium petroleum sulfonate having a molecular weight of about 500 and 67 weight percent of barium tert.-octyl phenol sulfide resin.

The treated product, after cooling to room temperature, was designated as Additive A. It had a phosphorus content of 3 weight percent, a sulfur content of 5.9 weight percent, and an S. U. S. viscosity at 210° F. of about 288.

*Additive B.*—This additive consisted of commercial chlorodibenzyl disulfide containing about 20 weight percent sulfur and 13 weight percent chlorine.

*Additive C.*—This material was a chlorinated camphene containing about 65 weight percent chlorine.

*Additive D.*—This was pentachlorophenol containing about 67% chlorine.

*Additive E.*—This was trichloroacetic acid containing about 65 weight percent chlorine.

### II. Description of oil base stocks

*Base Stock I.*—This was an SAE 90 grade gear oil consisting of about 47 weight percent of a deasphalted Mid-Continent crude residuum and 53 weight percent of a Mid-Continent acid-treated lubricating oil distillate. This mineral oil blend had an SUS viscosity of about 922 at 100° F. and about 81 at 210° F.

*Base Stock II.*—This was also an SAE 90-grade mineral oil prepared from solvent extracted Mid-Continent lubricating oils, and had SUS viscosities at 100° and 210° F. of about 864 and 79, respectively.

*Base Stock III.*—This was another SAE 90-grade mineral oil similar to Base Stock II. It had SUS viscosities at 100° and 210° F. of about 847 and 77, respectively.

### III. SAE test results

Oil blends containing either Additives A or B or a mixture of the two in Base Stock I were tested in the SAE extreme pressure testing machine according to the procedure designated CRC-L-17. The machine was operated at 1000 R. P. M. at a 14.7:1 rubbing ratio on the bearing cups. The minimum pressure that can be applied under these conditions is 10-15 scale pounds. In carrying out the test, pressure is increased until failure of the cups is obtained. The maximum reading before failure is designated as the SAE machine rating. The results of the tests are shown below in Table I.

TABLE I.—ADDITIVE IN OIL BLEND, WT. PERCENT

| Oil Blend      | Additive A<br>( $P_2S_5$ -trt.<br>Hydrocarbon) | Additive B<br>Chlorodibenzylsulfide | SAE Test<br>Results, Scale,<br>Pounds <sup>1</sup> |
|----------------|------------------------------------------------|-------------------------------------|----------------------------------------------------|
| 1 <sup>2</sup> | 0                                              | 0                                   | <15                                                |
| 2              | 0                                              | 1                                   | <15                                                |
| 3              | 10                                             | 0                                   | 78                                                 |
| 4              | 9                                              | 1                                   | 130                                                |

<sup>1</sup> Average of two runs.

<sup>2</sup> 100% Base Stock I.

The addition of 1% of the chlorodibenzylsulfide to the oil did not show a measurable improvement in the extreme pressure properties of the base oil. The addition of 10% of the phosphosulfurized hydrocarbon effected a substantial improvement, but an unexpected improvement of over 50 scale pounds was obtained by using a mixture of 9% phosphosulfurized hydrocarbon and 1% of the chlorodibenzylsulfide. This degree of improvement is all the more extraordinary in view of the fact that the sulfur and chlorine compound in the concentration used was ineffective when used alone. At most, the individual performance of the additives would indicate that the two additives together would impart an improvement of no more than that obtained by the addition of additive A alone.

### IV. Full scale gear tests

These tests were carried out on various blends of the additives and oil base stocks described in Examples I and II, above. The tests, designated as the High Speed-Low Torque Axle Test, CRC-L-19, and the High Torque-Low Speed Axle Test, CRC-L-20, were conducted in accordance with the U. S. Ordnance Specification MIL-L-2105. The base oils are incapable of passing either of these stringent tests. The oils containing photosulfurized hydrocarbons have in general excellent L-20 characteristics, but L-19 performance is frequently borderline or unsatisfactory. On the other hand, the conventional halogenated extreme pressure additives are generally either deficient in L-20 performance or are too corrosive to be used in high quality gear oils. In general, oils

containing the conventional halogenated organic com-

pounds are definitely deficient in L-19 performance, either with or without the addition of phosphosulfurized hydrocarbons. However, the combination of the phosphosulfurized additive and the sulfur and halogen-containing hydrocarbon was found to impart consistently superior L-19 performance to a variety of gear lubricants while, at the same time retaining excellent L-20 performance.

These effects are illustrated in Table II, below, showing the results of a series of runs carried out on the oil blends. Since emphasis has been placed on L-19 performance, this test is described briefly as follows: A new Chevrolet rear axle assembly lubricated by the oil being tested is operated under cyclic conditions of full throttle acceleration from 60 to 80 M. P. H. followed by closed throttle deceleration from 80 to 60 M. P. H. After ten such cycles, the gear teeth are inspected for scoring. If no scoring is noted, the oil passes the test, whereas the oil fails if the gear teeth scoring is light or severe. An oil is borderline if the scoring is slight.

TABLE II

| Oil Blend | SAE 90 Oil Base Stock | Additives used in Oil Blend, Weight Percent                             | Wt. Percent Chlorine in Oil | Full-Scale Gear Test |                 |
|-----------|-----------------------|-------------------------------------------------------------------------|-----------------------------|----------------------|-----------------|
|           |                       |                                                                         |                             | L-19                 | L-20            |
| 1.....    | I                     | None.....                                                               | Nil                         | Fail.....            | Fail.....       |
| 5.....    | I                     | 10% A (phosphosulfurized Hydrocarbon)                                   | Nil                         | do.....              | Pass.....       |
| 6.....    | I                     | 9% A, 1% B (Chlorodibenzyl disulfide)                                   | 0.13                        | Pass.....            | Do.....         |
| 7.....    | I                     | 7.4% A, 0.6% Zinc Stearate <sup>1</sup> , 2.0% C (Chlorinated Camphene) | 1.3                         | Fail.....            | Not Tested..... |
| 8.....    | I                     | 9.5% A, 0.5% D (Penta-chlorophenol)                                     | 0.33                        | do.....              | Do.....         |
| 9.....    | I                     | 9.7% A, 0.3% E (Trichloro-Acetic-Acid)                                  | 0.20                        | do.....              | Do.....         |
| 10.....   | <sup>2</sup> II       | 9% A, 1% B.....                                                         | 0.13                        | Pass.....            | Pass.....       |
| 11.....   | <sup>2</sup> III      | 10% A.....                                                              | Nil                         | Fail.....            | Do.....         |
| 12.....   | <sup>2</sup> III      | 9% A, 1% B.....                                                         | 0.13                        | Pass.....            | Do.....         |

<sup>1</sup> Added as corrosion inhibitor to offset corrosivity of Additive C.

<sup>2</sup> Base oils alone fail both L-19 and L-20 tests.

With reference to Table II, it is observed that all of the blends containing both Additives A and B passed both gear tests whereas oils containing only Additive A failed the L-19 test but passed the L-20 test. Furthermore, the oils containing Additives A and B were not corrosive to metals and met satisfactorily other specification requirements imposed on such gear oils.

The combination of sulfur-free, halogen-containing organic compounds with the phosphosulfurized hydrocarbon did not improve the oils sufficiently to meet the L-19 test, even though the halogen concentration in the oil blend was from almost 2 to 10 times greater than that in the oils of the present invention. In this connection, the chlorinated aliphatic compounds impart corrosive characteristics to the finished oils, and the use of an auxiliary corrosion inhibitor was needed in oil blend 7. What is claimed is:

An improved extreme pressure lubricating oil which comprises: a mineral oil having an SUS viscosity at 210° F. in the range of 50 to 150; 8 to 12 wt. percent of a dipentene-treated reaction product of a mineral lubricating oil and P<sub>2</sub>S<sub>5</sub>, formed at a temperature in the range of 200 to 600° F., and 0.5 to 2 wt. percent of chlorodibenzyl disulfide, the weight ratio of said dipentene-treated reaction product to said disulfide being in the range of 5:1 to 20:1.

## References Cited in the file of this patent

## UNITED STATES PATENTS

- |    |           |               |              |
|----|-----------|---------------|--------------|
| 30 | 2,153,482 | Prutton       | Apr. 4, 1939 |
|    | 2,450,405 | Berger et al. | Oct. 5, 1948 |
|    | 2,712,528 | Hill          | July 5, 1955 |